

## UNITED STATES PATENT OFFICE

2,610,949

## HYDRAULIC APPARATUS

Frank J. Sowa, Cranford, N. J.

No Drawing. Application September 13, 1948,

Serial No. 49,125

3 Claims. (Cl. 252—78)

1

This invention relates to a hydraulic apparatus by means of which mechanical forces are transmitted or absorbed. Thus, the apparatus of this invention may be in the form of a hydraulic brake, hydraulic clutch, shock absorber, dash pot, vibration dampener, artillery recoil mechanism, lifting jack, door check, etc.

Certain characteristics are required in devices which transmit or absorb mechanical forces using a fluid medium. Thus, the fluid contained therein must be stable both chemically and physically. The fluid must not react with the other parts of the device with which it comes into contact, that is, the fluid must not cause corrosion of exposed metal parts or effect any substantial swelling of rubber parts. In addition, the viscosity of the fluid should remain within the workable limits over a wide range of temperature, and should not have any tendency to gasify or solidify under higher and lower temperatures, respectively. The viscosity index of the fluid is of great importance, since the uniformity of operation of the device will depend in great part upon the uniformity of the viscosity of the fluid under temperature changes. The surface tension of the fluid contained in the device is also of importance, since the surface tension determines the facility with which the fluid wets the bearing surfaces and tends to creep into the engaging surfaces when the mechanism is static. Moreover, it is of importance that the fluid be one which shows a high resistance to hydrolysis under the conditions of use.

It is therefore the object of the present invention to provide a hydraulic device which meets the aforementioned requirements, particularly in that the force transmitting or absorbing fluid contained therein possesses a low pour point, high viscosity index, high surface tension, chemical inertness and substantial oiliness.

The aforementioned and other objects are accomplished in accordance with the present invention by employing in a conventional hydraulic apparatus a fluid comprising a compound of the generic formula



in which R, R' and R'' are alkyl radicals having from four to eighteen carbon atoms, cycloalkyl radicals having from five to eight carbon atoms, aryl hydrocarbon radicals having from six to eight carbon atoms, the benzyl or phenylethyl radical. Preferably, R, R' and R'' are either nor-

mal alkyl radicals having from four to six carbon atoms of the phenyl radical.

Thus, R, R' and R'' may suitably be the n-butyl, isobutyl, n-amyl, n-hexyl, 2-ethylhexyl, n-dodecyl, n-tetradecyl, stearyl, cycloamyl, cyclohexyl, o-methylphenyl, m-ethylphenyl, etc.

Suitable specific organosilicon monofluorides of the aforementioned generic formula are tri-n-butyl fluorosilane, tri-isobutyl fluorosilane, tri-n-amyl fluorosilane, triphenyl fluorosilane, tri-n-dodecyl fluorosilane, cyclohexyl di-n-butyl fluorosilane, phenyl di-isobutyl fluorosilane, tribenzyl fluorosilane, benzyl di-n-amyl fluorosilane, m-methylphenyl dicyclohexyl fluorosilane, etc.

15 The compounds of the aforementioned generic formula may be used alone as the hydraulic fluid or they may be used in admixture with up to about an equal weight of a comparable diluent which does not hydrolyze or oxidize appreciably under 20 the conditions of use. Such a diluent may be, for example, any of certain animal, vegetable or mineral oils, particularly castor oil or lubricating mineral oils. As a diluent there may also be used stable organic liquids having boiling points above 25 100° C., such as saturated aliphatic monohydric alcohols having at least four carbon atoms, such as fusel oil, 2-ethylhexanol, dodecyl alcohol, diacetone alcohol, the monoethyl ether of ethylene glycol, the monobutyl ether of ethylene glycol, the 30 monomethyl ether of diethylene glycol, the monobutyl ether of diethylene glycol, etc. Ethylene glycol and the diethyl and dibutyl ethers thereof are also examples of suitable diluents. In fact, any organic liquid which is miscible with the organosilicon monofluoride, which has a low viscosity and a relatively low vapor pressure at operating temperatures, which does not cause appreciable swelling of rubber and which does not react with metals may be used.

40 By way of illustrating the invention, a gun recoil shock absorber is filled with triamyl silicon fluoride, which remains fluid from —45° C. to 150° C. and does not hydrolyze under the conditions of use.

45 The present invention is directed to a hydraulic device which comprises essentially a cylinder or chamber enclosing a piston and a fluid contained in the cylinder or chamber, which fluid transmits or checks a mechanical force applied to the piston.

This application is a continuation-in-part of my copending application, Serial No. 463,684, filed October 28, 1942, which issued September 14, 1948, 55 as Patent No. 2,449,335.

## I claim:

1. A hydraulic apparatus comprising, in combination, a movable member and a liquid medium arranged in contact with said member, said liquid medium consisting essentially of at least one compound having the generic formula



in which R, R' and R'' are substituents selected from the group consisting of alkyl radicals having from four to eighteen carbon atoms, cycloalkyl radicals having from five to 8 carbon atoms, aryl hydrocarbon radicals having from six to 8 carbon atoms, the benzyl radical and the phenylethyl radical.

2. Apparatus as in claim 1 in which said liquid medium consists essentially of triamyl fluorosilane.

3. Apparatus as in claim 1 in which the liquid medium includes, in admixture with said compound, up to about an equal weight of said compound of an organic diluent having a boiling point above 100° C., which has a low viscosity, which does not cause an appreciable swelling of rubber, and which does not react with metals.

10

FRANK J. SOWA.

15

## REFERENCES CITED

The following references are of record in the file of this patent:

## 15 UNITED STATES PATENTS

| Number    | Name        | Date          |
|-----------|-------------|---------------|
| 2,205,183 | Woodhouse   | June 18, 1940 |
| 2,426,121 | Rust et al. | Aug. 19, 1947 |

20